

## UNITED STATES PATENT OFFICE

2,084,329

## NITRIDED ARTICLE OF MANUFACTURE

Joseph V. Emmons, Shaker Heights, Ohio, assignor to The Cleveland Twist Drill Company, Cleveland, Ohio, a corporation of Ohio

No Drawing. Application October 26, 1934,  
Serial No. 750,136

3 Claims. (Cl. 148—16)

This invention relates as indicated to nitrided articles of manufacture and this application is a continuation in part of my co-pending application Serial No. 655,861, filed February 8, 1933.

5 It has been known for quite some time that a hard case on a steel article may be secured by heating the metal in an atmosphere of nitrogen, ammonia usually being employed as the means for supplying the nitrogen. (See U. S. Patent No. 10,653,79 to Machlet.) It has been recognized, however, that a steel consisting of a simple alloy of iron and carbon does not absorb nitrogen during the customary nitriding process to an extent sufficient to make it useful as a body 15 material for the production of articles having a nitrided case.

Dr. Adolph Fry made a very important contribution to this art by his suggestion to add aluminum to the alloy being nitrided in order 20 to materially increase the rate of absorption of the nitrogen, thereby reducing the time required to secure sufficient penetration and further, a nitrided case secured in this manner is harder than a case possible on a simple alloy of iron and carbon. It has also been suggested (see Phillips U. S. Patent No. 1,697,083) to add molybdenum as an alloying element to the article being nitrided in order to make possible the rapid absorption of nitrogen and the production of a 25 satisfactory hard case of adequate depth. The nitrided surface or case formed on alloy steel articles of the type suggested by the prior art is usually satisfactory from the standpoint of its hardness and resistance to abrasion but a 30 principal difficulty has been encountered with the cracking and chipping of the hard and brittle nitrided surface layer or case due to the plastic deformation of the supporting steel core or body under working pressures.

35 The prior art has been primarily concerned with the production of hard nitrided cases upon core materials which were too weak and plastic to withstand the high chip pressures encountered with many cutting tools or the concentrated 40 loads frequently occurring in other forms of wear-resisting articles. This is particularly true because the temperatures at which the nitriding process is customarily effected (900° F. to 1100° F.) are such as to greatly reduce the hardness and 45 strength and increase the plasticity of the steels customarily employed as core materials if they have been previously hardened. A tool formed with a plastic core of insufficient hardness and strength, even though provided with a satisfactory nitrided case of sufficient hardness and capable of withstanding abrasion will, nevertheless, be useless for heavy duty work where the stresses to which the tool will be subjected are sufficient to deform the core to such an extent 50 that the nitrided case will crack or chip.

It is a principal object of my invention to provide an article of manufacture such as a tool or the like having a hard and brittle nitrided surface and a supporting body of great strength and hardness.

5 It is a further object of my invention to provide a supporting core, underneath the hard surface layer of a nitrided case, of greater resistance to plastic deformation than is possible with the so-called nitriding steels of the prior art. 10 This combination of properties makes possible a wearing surface which not only has great hardness and resistance to abrasion but which also has strong and rigid support from its underlying and supporting core. With this stronger support, 15 it is possible for the nitrided case to withstand greater pressures without being cracked and broken than is possible with the nitriding steels of the prior art.

20 Other objects of my invention will appear as the description proceeds.

To the accomplishment of the foregoing and related ends, said invention, then consists of the means hereinafter fully described and particularly pointed out in the claims.

25 The following description sets forth in detail certain products exemplifying my invention, such disclosed products constituting, however, but some of the various applications of the principles 30 of my invention.

35 As previously indicated, it is the principal object of this invention to provide an article of manufacture having a nitrided surface supported by an underlying core of exceptionally strong and hard steel capable of withstanding extreme operating stress without such plastic deformation as will cause a cracking or failure otherwise of the hard nitrided case.

40 The alloy steel compositions suitable for body material for nitrided articles in accordance with the present invention are characterized by a relatively high molybdenum content. The alloy steel compositions hereinafter referred to are all of such character that they may be properly defined as molybdenum tool steels. The following table 45 sets forth the broad ranges of percentages within which the several alloying elements may be present:—

|            | Percent       |    |
|------------|---------------|----|
| Carbon     | 0.25 to 1.30  | 50 |
| Manganese  | None to 2.00  |    |
| Silicon    | None to 3.00  |    |
| Chromium   | None to 15.00 |    |
| Tungsten   | None to 6.00  | 55 |
| Vanadium   | None to 5.00  |    |
| Molybdenum | 4.00 to 15.00 |    |

the remainder being substantially iron together with such other alloying elements and impurities as are sometimes found in alloy steels.

A somewhat narrower range of percentages within which the several alloying elements may be present is as follows:—

|             | Per cent      |
|-------------|---------------|
| 5 Carbon    | 0.50 to 1.00  |
| Manganese   | None to 2.00  |
| Silicon     | None to 3.00  |
| Chromium    | None to 5.00  |
| Tungsten    | None to 4.00  |
| 10 Vanadium | None to 3.00  |
| Molybdenum  | 6.00 to 12.00 |

the remainder being substantially iron together with such other alloying elements and impurities as are sometimes found in alloy steels.

In the foregoing tables giving ranges of percentages for the several alloying elements, the lower limits for manganese, silicon, chromium, vanadium and tungsten have been given as "none". As previously indicated, this invention relates to molybdenum tool steels. The tables of percentages previously given are to be interpreted, therefore, as covering only those steels in which the elements manganese, silicon, chromium, vanadium and tungsten are present in a total amount not less than 3.00%, although any one or more of such elements may be entirely absent.

An illustrative specific alloy steel composition which is suitable for body material for nitrided articles is as follows:

|            | Per cent   |
|------------|------------|
| Carbon     | about 0.61 |
| Manganese  | do 0.23    |
| 35 Silicon | do 0.29    |
| Chromium   | do 3.65    |
| Tungsten   | do 1.69    |
| Vanadium   | do 1.00    |
| Molybdenum | do 6.67    |

40 the balance being iron, together with such impurities as are usual in alloy steels.

This steel possesses properties which approach those of high speed steel, although the amount 45 of alloy present is much less than is usually employed in such steels. With this composition a hardening temperature as high as 2200° F. may be employed together with drawing temperatures up to 1150° F. Tools made from this steel such 50 as twist drills, possess great strength and cutting quality, these properties being maintained at operating temperatures up to red heat.

After hardening at 2200° F. and nitriding, a 55 steel according to the last above enumerated composition has a surface layer of great hardness supported by a rigid core of great strength and of a hardness sufficient to itself function as a cutting tool.

60 Still another example of a specific alloy steel composition which is suitable for body material for nitrided articles is as follows:

|             | Per cent   |
|-------------|------------|
| Carbon      | about 0.66 |
| 65 Chromium | do 4.26    |
| Tungsten    | do 0.10    |
| Vanadium    | do 1.14    |
| Molybdenum  | do 10.19   |

70 the balance being iron, together with such other alloying elements and impurities as are usual in alloy steels.

A still further example of a specific alloy steel composition successfully utilized for the purposes 75 of the invention is as follows:

|            | Per cent   |
|------------|------------|
| Carbon     | about 0.77 |
| Chromium   | do 3.85    |
| Tungsten   | do 1.99    |
| Vanadium   | do 1.03    |
| Molybdenum | do 11.15   |
| Cobalt     | do 9.06    |

the balance being iron and such other alloying elements and impurities as are usual in alloy 10 steels. The steel of the last above mentioned composition is of the type in which molybdenum is the principal alloying constituent and contains about one fourth as much tungsten as molybdenum. It also contains a considerable percentage of cobalt. The body of this steel underneath the nitrided case has exceptional hardness and strength due to its great resistance to tempering. Its microstructure, after nitriding, is still predominantly martenitic. 20

Another example of a specific alloy steel composition is as follows:—

|            | Per cent   |
|------------|------------|
| Carbon     | about 0.87 |
| Manganese  | do 0.12    |
| 35 Silicon | do 0.40    |
| Chromium   | do 3.35    |
| Vanadium   | do 1.31    |
| Molybdenum | do 7.65    |
| Nickel     | do 2.17    |

the balance being iron together with such other alloying elements and impurities as are usual in alloy steels.

This steel is notable for a substantial nickel 35 content. It has an unusual resistance to tempering, maintaining a high hardness after tempering treatments which approach tool steel annealing conditions. It takes a nitrided case of great hardness and depth.

Another example of a specific alloy steel composition is as follows:—

|            | Per cent |
|------------|----------|
| Carbon     | 1.29     |
| Manganese  | 0.11     |
| 35 Silicon | 0.47     |
| Chromium   | 3.29     |
| Tungsten   | 1.61     |
| Vanadium   | 3.29     |
| Molybdenum | 8.04     |

the balance being iron together with such other alloying elements and impurities as are usual in alloy steels.

This steel is notable for high contents of carbon 55 and vanadium. It takes a nitrided case of great depth and hardness.

As previously indicated, the compositions enumerated herein are such that the alloying elements are present in such proportions as to stabilize the martenitic structure of the steels so that it is possible to temper the steel simultaneously with the nitriding operation without losing a prohibitive amount of hardness and strength.

The compositions hereinbefore enumerated are sufficiently hard and of such great strength so that when tools and like articles made therefrom are subjected to severe working stresses the supporting core for the nitrided case will not be deformed and the case will accordingly be preserved against cracking and chipping. 65

The utility of such nitrided cases is not confined to the cutting portion of tools but may be widely extended to such purposes as pilots, guides, 75

or other articles and parts which are subject to abrasion or wear.

As an example, nitrided parts so supported may be used in complex tools of which the principal cutting or wear-resisting action is performed by parts of non-ferrous, hard metal compositions such as tungsten or tantalum carbides. When so used, it has been found that the nitriding operation can be carried out without material damage to the working parts of the hard metal composition and with actual improvement of the strength and toughness of the tool body due to the desirable tempering action.

As is well known to those familiar with the art, any specification for a particular alloy composition must permit of certain variations due to the fact that in making up the composition, it is extremely difficult, if not impossible, to commercially produce a composition exactly like a given specification. It is to be understood, therefore, that throughout the description and claims where I have used figures to denote definite amounts and ranges, such amounts and ranges are to be construed to include the range of variations usually permissible in making up alloy compositions to given specifications.

Other forms may be employed embodying the features of my invention instead of the one here explained, change being made in the form or construction, provided the elements stated by any of the following claims or the equivalent of such stated elements be employed.

I, therefore, particularly point out and distinctly claim as my invention:

1. The method of producing a metallic article such as a tool, having great body strength and a hard wear-resistant surface, which comprises forming the body of such article of a ferrous alloy characterized by the presence therein of:

Carbon from about 0.25% to about 1.30%  
Molybdenum from about 4.00% to about 15.00%

and a total of not less than 3% of at least one of the following elements individually present in amounts not exceeding the following percentages:

|           | Per cent |
|-----------|----------|
| Manganese | 2.00     |
| Silicon   | 3.00     |
| Chromium  | 15.00    |
| Tungsten  | 6.00     |
| Vanadium  | 3.00     |

hardening said body by heat treatment, and by subsequent heat treatment tempering the core and nitriding the surface of said body, an effect

of the presence of the named alloying elements in said body being to prevent the decomposition during said tempering and nitriding of a substantial portion of the martensitic structure of said body.

2. The method of producing a metallic article such as a tool, having great body strength and a hard wear-resistant surface, which comprises forming the body of such article of a ferrous alloy characterized by the presence therein of the following elements within the percentages given:

|            | Per cent                         |
|------------|----------------------------------|
| Carbon     | from about 0.50% to about 1.00   |
| Molybdenum | from about 6.00% to about 12.00  |
| Manganese  | from an effective amount to 2.00 |
| Silicon    | from an effective amount to 3.00 |
| Chromium   | from an effective amount to 5.00 |
| Tungsten   | from an effective amount to 4.00 |
| Vanadium   | from an effective amount to 3.00 |

with the combined manganese, silicon, chromium, tungsten and vanadium content being equal to at least 3%, hardening said body by heat treatment, and by subsequent heat treatment tempering the core and nitriding the surface of said body, an effect of the presence of the named alloying elements in said body being to prevent the decomposition during said tempering and nitriding of a substantial portion of the martensitic structure of said body.

3. The method of producing a metallic article such as a tool, having great body strength and a hard wear-resistant surface, which comprises forming the body of such article of a ferrous alloy characterized by the presence therein of the following elements within the percentages given:

|            | Per cent   |
|------------|------------|
| Carbon     | about 0.77 |
| Chromium   | do 3.85    |
| Tungsten   | do 1.99    |
| Molybdenum | do 11.15   |
| Vanadium   | do 1.03    |
| Cobalt     | do 9.06    |

hardening said body by heat treatment, and by subsequent heat treatment tempering the core and nitriding the surface of said body, an effect of the presence of the named alloying elements in said body being to prevent the decomposition during said tempering and nitriding of a substantial portion of the martensitic structure of said body.

JOSEPH V. EMMONS. 55